

Patented Mar. 2, 1937

2,072,665

## UNITED STATES PATENT OFFICE

2,072,665

## BLEACHING PROCESS

Donald J. Campbell and Le Roy P. London,  
Niagara Falls, N. Y., assignors to E. I. du Pont  
de Nemours & Company, Wilmington, Del., a  
corporation of Delaware

No Drawing. Application September 25, 1934,  
Serial No. 745,452

13 Claims. (Cl. 8-2)

This invention relates to a method of bleaching and more particularly to a process for bleaching cattle hair, fur or any dark animal fiber in order to produce a product of satisfactory light color and undamaged texture.

One of the objects of this invention is to employ satisfactorily in the bleaching of dark animal fiber, such as cattle hair or fur which usually contains a residual depilatory, an alkaline hydrogen peroxide solution or an alkaline solution yielding hydrogen peroxide under the conditions of use. Another object of this invention is to include as a pre-treatment step in the bleaching operation a treatment which will remove dark inorganic coloring, such as that caused by iron, from an animal fiber as cattle hair which may be stained a reddish or dark brown color as a result of iron present therein. Still another object of this invention is to convert these iron compounds present in an animal fiber such as cattle hair into a condition in which they may be removed readily therefrom before subjecting the cattle hair to the subsequent alkaline peroxide bleach.

Ordinarily, cattle hair contains residues from the depilatory agent which has been employed to remove the hairs from the body of the animal. The most usual depilatory agents are calcium compounds, such as calcium sulfide and calcium hydroxide. We have found that when hydrogen peroxide or a compound yielding hydrogen peroxide is employed as the bleaching agent, and cattle hair is introduced into the bleach bath without preliminary treatment of any sort, the bleaching cost is very high. After considerable experimentation, we have found that the presence of iron and calcium in the cattle hair or other animal fiber being treated, conjointly act as a catalytic agent of high efficacy for the decomposition of hydrogen peroxide. Thus, when animal fiber containing residues of the depilatory agents and iron is introduced directly into an alkaline peroxide bleach bath, a large part of the peroxide loss is caused by the catalytic action of the elements mentioned and but little of the chemical is used up in effecting the bleaching. An object of this invention, therefore, is to develop a process which will give the most satisfactory degree of whiteness for a given chemical cost. Previously, the same degree of whiteness attained by the use of our process has been obtainable, but only by the use of much larger quantities of hydrogen peroxide, and a consequent increased chemical cost. These and still other objects of our invention will be apparent from the proce-

dure hereinafter described which is the best method known to us for satisfactorily bleaching such materials as cattle hair and other animal fibers by the use of an alkaline hydrogen peroxide bleach without the chemical cost running beyond that expense which is economical in commercial bleaching.

The animal fiber is first subjected to the action of a reducing agent, such as sodium bisulphite,  $\text{NaHSO}_3$ , for the purpose of converting any iron compounds present therein or thereon which may cause part of the reddish or dark coloration thereof and which are very undesirable because of their catalytic effect in decomposing hydrogen peroxide with consequent losses of peroxide, from the ferric state to the ferrous state. Sulfur dioxide may be used to accomplish this reaction but we prefer to use the sodium-hydrogen salt of sulfurous acid, sodium bisulfite. Preferably, the animal fiber, whether it be cattle hair or some other dark colored fiber, is steeped in a bath comprising from two to eight pounds of sodium bisulphite per one-hundred gallons of bleaching solution. To the bath, dilute sulfuric acid in concentration equivalent to 0.25% or less is also added, as the salt exerts its reducing action preferably in acid media. If desired, sodium hydrosulfite,  $\text{Na}_2\text{S}_2\text{O}_4$ , in equivalent amount may be used as a reducing compound and this salt acts best in alkaline solutions. The time of treatment may vary from 15 minutes to 1 hour, although we have found 30 minutes to be a most satisfactory time for the usual commercial cattle hair. The temperature may be room temperature or may be an elevated temperature, preferably not higher than  $180^\circ \text{ F}$ . Above this temperature, sulfur dioxide is freely evolved from the sodium bisulfite and besides escaping into the atmosphere may also have a deleterious effect on the fiber being bleached. The presence of an excess of  $\text{SO}_2$  may cause harshening of the fiber, especially in those cases in which the total quantity of  $\text{SO}_2$  evolving materials is large. We prefer that the temperature be maintained at about  $140^\circ \text{ F}$ . as we have found that temperature most suitable for our preferred bleach bath which contains two pounds of sodium bisulfite per one-hundred gallons of bleaching solution and enough sulfuric acid to render the acid concentration in the bleach bath approximately 0.25%.

The sodium bisulfite treatment or treatment with any other reducing agent, such as sulfur dioxide, is essentially for the purpose of reducing the ferric compounds present in the material to the ferrous state, in which state they may be

readily removed by means of an acid. We prefer to use for this purpose an inorganic mineral acid, and preferably hydrochloric acid, although organic acids may be used. Concentrations 5 from 0.5% to 5% by weight, made up by using c. p. hydrochloric acid of specific gravity of 1.18, are most suitable. Hydrochloric acid is perhaps the cheapest of the mineral acids and we have found our process to 10 give results of entire satisfaction with a solution of that acid of 2% concentration. The treatment time may vary from 15 to 30 minutes but we have found that under most conditions, one-quarter of an hour of treatment is all that is 15 necessary to remove substantially all of the iron. Here again, an elevated temperature may be used and in general, any temperature from room temperature to 140° F. has been found suitable. Under certain conditions, the acid may be boiled 20 with the animal fiber, as when cattle hair is being treated, but ordinarily, boiling will not be necessary unless the fiber is extremely discolored. This treatment also removes any lime compounds which may be present on the hair or fibers, which 25 is very desirable, for as previously pointed out, iron and lime together constitute an agent for catalytic decomposition of hydrogen peroxide which is of far superior action to that of compounds of either element when present alone.

30 Following the acid treatment for the removal of iron from the animal fiber, which iron has preferably been converted to the ferrous state, in which condition it is more readily removed, the next step in our process involves neutralizing 35 the acid. For this purpose, we prefer to treat the cattle hair with a solution containing from two to six pounds of sodium carbonate,  $\text{Na}_2\text{CO}_3$ , per one-hundred gallons of solution, although other alkalining agents, such as caustic alkali or 40 sodium silicate, may be used. We prefer a solution containing four pounds per one-hundred gallons of solution for the usual commercial cattle hair. The treatment period necessary ranges from 15 minutes to 1 hour with  $\frac{1}{2}$  hour being the 45 preferred time of treatment. Here again, either room temperature or an elevated temperature up to 140° F. may be employed and in general, we prefer to use a temperature of 120° F.

50 After neutralizing the acid, the cattle hair is then treated with an additional amount of sodium carbonate for the purpose of scouring the fiber. This treatment also serves to remove the suint or waxy and oily residue caused by animal perspiration and deposited on the fiber. This 55 solution should preferably consist of from two to four pounds of sodium carbonate per one-hundred gallons of solution, two pounds having been found most suitable for ordinary commercial cattle hair. The treatment time should range from 15 minutes to 1 hour, one-half hour being preferred; the temperature may be either room temperature or an elevated temperature such as 140° F. The 60 temperature of 120° F. has been found most generally suitable.

65 In place of the sodium carbonate, a soap may be used which will also effectively scour the fiber and remove suint. Ordinarily, it may be more advantageous in commercial bleacheries to use 70 both sodium carbonate and a soap in the scouring bath for the removal of suint.

75 The treatment for the neutralization of the acid and that for the purpose of scouring the fiber may also advantageously be combined into one treatment, under some circumstances, by the use

of an increased amount of sodium carbonate or other suitable alkalinizing agent. We have found it most satisfactory in general, however, first to neutralize the acid by the use of an alkalinizing agent and then to complete the scouring by the 5 use of a separate treatment step and a fresh solution containing sodium carbonate and/or a soap. One reason for this is that otherwise inert salts formed by neutralization of the acid will be present in the treating solution and may interfere with successful scouring. However, the chief reason is that ordinarily if both steps are carried out in a single operation, i. e., the step of neutralization and the step of scouring, the concentration of hydroxyl ion in the solution will 10 become so high as to produce deleterious effects usually termed "harshening" on the fiber being treated. Consequently, we prefer to carry out each operation separately although in commercial bleacheries, expediency may sometimes dictate the use of single operation even at the risk of some minor damage resulting to the fiber.

15 After the removal of the iron and scouring of the fiber to remove suint and other material readily removable by means of an alkaline or soapy 20 scouring treatment, the fiber is in condition for bleaching with hydrogen peroxide or any material yielding hydrogen peroxide, such as an alkali metal peroxide. We have found an alkaline 25 bleaching solution more suitable than an acid 30 bleaching bath and in general, we have found most desirable alkaline solutions which contain stabilizing and buffering agents, such as sodium pyrophosphate, sodium silicate, and borax. In 35 general, we have found alkaline bleaching solutions made up as follows and containing hydrogen peroxide as the active bleaching agent most suitable:

#### Solution A

40

2 lbs. of borax per 100 gals. of solution.

2 lbs. of sodium pyrophosphate per 100 gals. of solution.

2 lbs. of sodium silicate per 100 gals. of solution.

45

3 to 12 gals. of 100-volume hydrogen peroxide per 100 gals. of solution.

(Preferably, 5 gals. of 100-volume  $\text{H}_2\text{O}_2$  per 100 gals. of solution are used for the ordinary commercial cattle hair.)

#### Solution B

50

2 lbs. of borax per 100 gals. of solution.

4 lbs. of sodium pyrophosphate per 100 gals. of solution.

55

3 to 12 gals. of 100-volume hydrogen peroxide per 100 gals. of solution.

(Preferably, 5 gals. of 100-volume  $\text{H}_2\text{O}_2$  per 100 gals. of solution are used for the commercial cattle hair ordinarily encountered).

60 The treatment time may vary from 8 to 24 hours and usually, the longer the fiber is immersed in the bleaching solution, the better will 65 be the degree of whiteness produced. The temperature may range from room temperature to an elevated temperature, such as 140° F. as a maximum and ordinarily, a higher temperature up to 140° F. produces an enhanced bleaching 70 action without deleterious effect on the cattle hair or other fiber.

75 By the use of our process, it is possible to produce a bleached animal fiber of lighter color than was formerly obtainable by any of the

8. BLEACHING & DYEING; FLUID  
TREATMENT & CHEMICAL MODIFI-  
CATION OF TEXTILES & FIBERS,

2,072,665

3

110

now known methods having approximately the same chemical costs. While it is possible with the expenditure of considerable bleaching agent to produce an animal fiber of a high degree of 5 whiteness, formerly it was not possible economically to utilize hydrogen peroxide in the bleaching of these fibers. Our process permits the obtainment of a satisfactory lightened color with animal fiber, such as cattle hair, at a chemical 10 cost which is well within the limits permitted in commercial bleaching operations.

As will be apparent, our improved process results from the elimination of iron and/or calcium compounds from the fiber previous to 15 bleaching which compounds previously destroyed a large amount of hydrogen peroxide by reason of their catalytic action with a consequent increase in the amount of peroxide essential to bleach the fiber, thereby resulting in an increased 20 chemical cost. The procedures and amounts given above are to be considered as illustrative and not as restrictive, and various changes may be made in the precise temperatures, times and amounts without departing from the spirit of 25 our invention. In short, changes may be made which will not employ the precise amounts and conditions specified but will still fall within the scope of our invention as defined by the appended claims.

30 Wherever, in the following claims, hydrogen peroxide is referred to, we intend to include in the scope of that term any material or materials which, under the conditions of the process, will yield hydrogen peroxide or a solution thereof.

35 We claim:

1. A process of bleaching animal fiber which comprises the steps of treating the unbleached fiber with a reducing agent, capable of evolving sulfur dioxide, then subjecting the fiber to the 40 action of an acid solvent for the soluble reduced compounds resulting from the action of the reducing agent, and finally subjecting the fiber to the action of a dilute alkaline bleaching solution of hydrogen peroxide.

45 2. A process of bleaching animal fiber which comprises the steps of treating the unbleached fiber with a reducing agent capable of evolving sulfur dioxide, then subjecting the fiber to the action of a dilute acid and subsequently bleaching the fiber with a dilute hydrogen peroxide bleaching solution.

50 3. A process of bleaching animal fiber which comprises the steps of treating the unbleached fiber with a reducing agent capable of evolving sulfur dioxide, then subjecting the fiber to the 55 action of a mineral acid, and finally bleaching the fiber with a dilute solution of hydrogen peroxide.

60 4. A process of bleaching animal fiber which comprises the steps of treating the unbleached fiber with a reducing agent selected from the group which consists of sodium bisulfite and sodium hydrosulfite, then subjecting the fiber to the 65 action of a mineral acid, and subsequently bleaching with a dilute hydrogen peroxide solution.

65 5. A process of bleaching animal fiber which comprises the steps of treating the unbleached fiber with a reducing agent selected from the group which consists of sodium bisulfite and sodium hydrosulfite, then subjecting the fiber to the 70 action of a mineral acid, neutralizing any acid present on the fiber, and subsequently bleaching with a dilute solution of hydrogen peroxide.

6. A process of bleaching animal fiber which comprises the steps of treating the unbleached fiber with a reducing agent, capable of evolving sulfur dioxide, then subjecting the fiber to the action of a dilute mineral acid, neutralizing, 5 scouring the fiber with an alkaline scour, and finally bleaching the fiber with a dilute alkaline solution of hydrogen peroxide.

7. A process of bleaching animal fiber which comprises the steps of treating the unbleached fiber first with a solution of a reducing agent selected from the group which consists of sodium bisulfite and sodium hydrosulfite, then adding a mineral acid, neutralizing any acid on the fiber, treating said fiber with an alkaline scour, and 15 finally treating said fiber with hydrogen peroxide for the purpose of bleaching said fiber in a dilute alkaline active oxygen bleach bath.

8. A process of bleaching animal fiber which comprises the steps of treating the unbleached fiber with sodium bisulfite, adding hydrochloric acid to dissolve out the undesired discoloring compounds, neutralizing, adding sodium carbonate for the purpose of scouring the fiber, and finally adding hydrogen peroxide to said solution, 20 thereby effecting bleaching of the animal fiber in a dilute alkaline hydrogen peroxide bleaching solution.

9. A process of bleaching animal fiber which comprises the steps of treating unbleached fiber 30 with sodium bisulfite, subjecting the fiber to the action of hydrochloric acid, scouring the fiber with a scouring solution containing sodium carbonate, and subsequently bleaching the fiber with a dilute alkaline solution of hydrogen peroxide. 35

10. A process of bleaching cattle hair which comprises the steps of adding sodium bisulfite to a solution containing the cattle hair suspended therein for the purpose of reducing iron compounds present in said cattle hair, adding a dilute 40 mineral acid to said liquor for the purpose of dissolving out said reduced compounds formed as a result of the treatment with a reducing agent, neutralizing said solution, adding sodium carbonate thereto and heating for the purpose of 45 scouring the cattle hair, and subsequently adding hydrogen peroxide to said liquor for the purpose of bleaching said cattle hair in a dilute alkaline active oxygen yielding bath.

11. A process of bleaching cattle hair which 50 comprises subjecting the cattle hair to the action of a sodium bisulfite solution having a concentration of 0.25%-1% at a temperature within the range, room temperature to 180° F. for a period of 15 minutes to 1 hour, then subjecting the 55 cattle hair to the action of a solution of hydrochloric acid of a concentration ranging from  $\frac{1}{2}\%$ -5% at a temperature ranging from room temperature to 180° F. for a period of 15 to 30 minutes, then subjecting the cattle hair to the 60 action of a solution of sodium carbonate ranging in concentration from 0.25% to 0.75% for a period of 15 minutes to 1 hour at a temperature ranging from room temperature to 140° F., then subjecting said cattle hair to the action of a solution of sodium carbonate ranging in concentration from 0.25% to 0.50% for 15 minutes to 1 65 hour at a temperature ranging from room temperature to 140° F., and finally bleaching said cattle hair in a dilute alkaline solution of hydrogen peroxide which contains stabilizing agents. 70

12. A process of bleaching cattle hair which comprises treating said cattle hair with a solution of sodium bisulfite of approximately 0.25% concentration for half an hour at a temperature 75

of substantially 120° F., then treating the cattle hair with a solution of hydrochloric acid of approximately 2% concentration at room temperature for approximately 15 minutes, then treating the cattle hair with a solution of sodium carbonate of approximately 0.5% concentration for 30 minutes at a temperature of approximately 120° F., then treating said cattle hair with a solution of sodium carbonate of approximately 0.25% concentration for half an hour at a temperature of substantially 120° F., and then bleaching said cattle hair with a dilute alkaline solution of hydrogen peroxide.

13. A process of bleaching cattle hair which comprises subjecting said cattle hair to the action of a reducing agent selected from the group which consists of sodium bisulfite and sodium hydrosulfite, subjecting said cattle hair to the action of a dilute mineral acid, subjecting said cattle hair to the action of an alkaline scour, and then bleaching said cattle hair in a dilute solution of hydrogen peroxide.

5

10

DONALD J. CAMPBELL.  
LE ROY P. LONDON.